# EUROPEAN PATENT APPLICATION

(11) **EP 3 964 661 A1**
(43) Date of publication of application: **09.03.2022**
(21) Application number: 20250002.1
(22) Date of filing: 08.09.2020
(51) Int. Cl.: E04B 5/04, E04B 5/32, E04C 5/08, E04C 5/01, E04C 5/07

(54) **POST-TENSIONED CONCRETE WITH FIBERS FOR SLABS ON SUPPORTS**

(71) Applicant: NV Bekaert SA, 8550 Zwevegem (BE); CCL Stressing International Limited, West Yorkshire LS11 5BP (GB)
(72) Inventor: Thooft, Hendrik, 9700 Welden (BE); Hayek, Carol, Leeds, LS11 SBP (GB)
(74) Representative: Messely, Marc

(57) **Abstract**

The present invention concerns a concrete slab resting on at least two supports, the slab comprising conventional concrete and a combined reinforcement of both draped post-tension steel strands and fibers,
said post-tension steel strands
- having a diameter ranging from 5 mm to 20 mm,
- having a tensile strength higher than 1700 MPa,
said fibers being either steel fibers and being present in a dosage ranging from 10 kg/m³ to 75 kg/m³ or being macro-synthetic fibers and being present in a dosage ranging from 1,5 kg/m³ to 9,0 kg/m³,
whereby the slab and the supports are fully connected, partially connected or fully disconnected.

## Description

### Technical Field

The invention relates to a concrete slab comprising conventional concrete and a combined reinforcement of both post-tension steel strands and fibers on at least two supports.

### Background Art

Post-tensioned concrete is a variant of pre-stressed concrete where the tendons, i.e. the post tension steel strands, are tensioned after the surrounding concrete structure has been cast and hardened. It is a practice known in the field of civil engineering since the middle of the twentieth century.

Steel fiber reinforced concrete is concrete where the reinforcement is provided by short pieces of steel wire that are spread in the concrete. US-A-1,633,219 disclosed the reinforcement of concrete pipes by means of pieces of steel wire. Other prior art publications US-A-3,429,094, US-A-3,500,728 and US-A-3,808,085 reflect initial work done by the Batelle Development Corporation. The steel fibers were further improved and industrialized by NV Bekaert SA, amongst others by providing anchorage ends at both ends of the pieces of steel wire, see US-A-3,900,667. Another relevant improvement was disclosed in US-A-4,284,667 and related to the introduction of glued steel fibers in order to mitigate problems of mixability in concrete. Flattening the bent anchorage ends of steel fibers, as disclosed in EP-B1-0 851 957, increased the anchorage of the steel fibers in concrete. The supply of steel fibers in a chain package was disclosed in EP-B1-1 383 634.

Both reinforcement techniques, post-tensioned concrete and fiber reinforced concrete such as steel fiber reinforced concrete not only exist as such but also in combination. The purpose was to combine the advantages of both reinforcement types to obtain an efficient and reliable reinforced concrete slab.

Prior art concrete slabs with combined reinforcement of both post-tension strands and fibers suffer from an overdesign or from a complex design. In an attempt to stay on the very safe side and to meet the specifications, the dosage of steel fibers is often that high that problems such as ball forming occur during mixing of the steel fibers in the non-cured concrete, despite the existence of prior art solutions. Alternatively, or in addition to this, the distance between two neighbouring post-tension strands or between two neighbouring bundles of post-tension strands cannot exceed certain maximum spacing, causing a lot of labour when installing the post-tension strands, attaching anchors and applying tension. In yet other prior art embodiments the composition of the concrete is such that shrinkage during curing is limited, i.e. for example a low shrinkage concrete or a shrinkage compensating concrete composition may be selected.

An example of a complex design of a concrete slab with reinforcement by both post-tension steel strands and steel fibers is disclosed in NZ-A-220 693. This prior art concrete slab has an under and upper skin layer with steel fibers with a core layer in-between with post-tension tendons.

The present invention may thereby improve the span of the slabs and/or reduce the thickness of the slab and/or the present invention may contribute to reduce the amount of concrete for a given slab thickness or a given span. Furthermore, the present invention may allow for easier and/or faster installation. In addition, the present invention may allow for the slabs to be structural slabs that can for example contribute to structural integrity of a building. The present invention may further contribute to increase the structural capacity for flexure, deflection, shear, punching shear, structural integrity, temperature resistance and/or resistance to shrinkage. The present invention especially allows to combine for example improved shear or punching shear resistance with improved flexural capacity. Furthermore, the present invention advantageously allows for example that post tensioning strands can remain unstressed, even without partial stressing, without the need for shrinkage reinforcement.

### Disclosure of Invention

It is a general aspect of the invention to avoid the disadvantages of the prior art.

It is a further general aspect of the invention to avoid overdesign.

It is another aspect of the invention to provide a combination reinforcement of both post-tension strands and fibers to reinforce concrete slabs on supports efficiently and effectively.

It is still another aspect of the invention to provide a combination reinforcement of both post-tension strands and fibers for conventional concrete slabs on supports.

According to the invention, there is provided a concrete slab resting on at least two supports, the slab comprising conventional concrete and a combined reinforcement of both draped post-tension steel strands and fibers, said post-tension steel strands
- having a diameter ranging from 5 mm to 20 mm,
- having a tensile strength higher than 1700 MPa,
said fibers being either steel fibers and being present in a dosage ranging from 10 kg/m³ to 60 kg/m³ or being macro-synthetic fibers and being present in a dosage ranging from 1,5 kg/m³ to 9,0 kg/m³,
whereby the slab and the supports are fully connected, partially connected or fully disconnected.

The tendons or post-tension steel strands having a diameter ranging from 5 mm to 20 mm, e.g. from 6 mm to 20 mm, e.g. from 6,5 mm to 18,0 mm. The post-tension steel strands have a tensile strength higher than 1700 MPa, e.g. higher than 1800 MPa, e.g. higher than 1900 MPa, e.g. higher than 2000 MPa.

The tendons or post-tension steel strands may be bonded or unbonded. In addition, the steel strands may preferably for example be present in bundles.

Particularly with a view to be used as post-tension steel strand, the steel strand preferably has a low relaxation behaviour, i.e. a high yield point at 0,1% elongation. The yield point at 0,1% can be considered as the maximum elastic limit. Below the yield point, the post-tension strand will remain in elastic mode. Above the yield point, the post-tension strand may start to elongate in plastic mode, i.e. an elongation that is not reversible. Preferably, the ratio of the yield strength R_{p0,1} to the tensile strength Rₘ is higher than 0,75.

Low relation post-tension steel strands may have relaxation losses of not more than 2.5 % when initially loaded to 70 % of specified minimum breaking strength or not more than 3.5 % when loaded to 80 % of specified minimum breaking strength of the post-tension steel strand after 1000 hours.

The fibers can be steel fibers and are present in a dosage ranging from 10 kg/m³ to 40 kg/m³, alternatively from ≥ 25 kg/m³ to 75 kg/m³ or 20 kg/m³ to 30 kg/m³, furthermore from > 40 kg/m³ to 60 or 65 kg/m³.

The fibers can be macro-synthetic fibers and are present in a dosage ranging from 1,5 kg/m³ to 9 kg/m³, e.g. from 2,5 kg/m³ to 7 kg/m³, e.g. from 3,5 kg/m³ to 5,0 kg/m³.

The fibers are present in all parts of the concrete slab, i.e. the concrete slab is preferably a monolithic slab and the fibers are substantially homogeneously or homogeneously distributed in the concrete slab. Substantially homogeneously may thereby mean for example except for a very thin (preferably below 10 mm, further preferred below 6 mm) upper skin layer that is applied to provide a flat and wear resistant surface to the slab and to avoid fibers from protruding. This may especially allow to contribute for example to improving punching shear. In an embodiment, the slab may preferably be cast in one or multiple steps, preferably in one step.

Dosages of fibers of 10 kg/m³ to 40 kg/m³ in case of steel fibers and 1,5 kg/m³ to 9 kg/m³ in case of macro-synthetic fibers are low to moderate in comparison with prior art dosages of more than 40 kg/m³ or more than 9 kg/m³. Such low to moderate dosages may for example further allow integrating the fibers in a more homogeneous way in the concrete and facilitate the mixing of the fibers in the concrete.

The conventional concrete preferably has a characteristic compressive cube strength or comparable cylinder strength 25 N/mm² or higher, preferably 28 N/mm² or higher, further preferred 30 N/mm² or higher. More preferably, the conventional concrete has a strength equal to or higher than the strength of concrete of the C20/25 strength classes as defined in EN206 or equivalent national code requirements and smaller than or equal to the strength of concrete of the C50/60 strength classes as defined in EN206. These types of concrete are widely available and avoid adding ingredients that reduce the shrinkage during hardening. For the avoidance of doubt, self-compacting concrete is considered as conventional concrete. In a preferred embodiment, the slab does not contain any further reinforcement elements, such as rebars or steel nets or steel mesh beside steel fibers and post-tensioning steel strands, especially there may no rebars neither at the top nor at the bottom, further preferred there may also be for example even no rebars at the supports. It is thereby especially advantageous that the slabs according the present invention can act as structural slabs, especially for example to contribute to the structural integrity of a building.

In a preferable embodiment of the invention, the fibers are steel fibers and have a straight middle portion and anchorage ends at both ends.

Most preferably the tensile strength of the middle portion is above 1400 MPa, preferably above 1500 MPa, preferably above 1700 MPa, further preferred above 1900 MPa, even further preferred above 2000 MPa.

The anchorage ends preferably each comprise three or four bent sections. Examples of such steel fibers are disclosed in EP-B1-2 652 221 and in EP-B1-2 652 222.

In an embodiment of the invention, the supports may be concrete supports, masonry supports, steel supports or supports combining concrete, masonry and/or steel.

In an embodiment of the invention, the supports may be part of a foundation, preferably located underneath the slab and/or away from the foundation, or preferably, the supports may not be part of a foundation. In case the supports are part of a foundation of a building, they may be preferably in contact with the soil or ground. On the other hand, in the case the supports are not part of a foundation of a building, the slab may preferably be a so-called elevated slab, they may especially be part of a multi-story building above or below the ground level. Elevated slabs and/or their supports may thereby preferably not be contact with the soil or ground, preferably elevated slabs (in contrast to slabs laid on the ground) may thereby also not be uniformly supported along the slab but rather punctually supported at the supports. It is thereby especially advantageous that the slabs according the present invention can act as or be structural slabs, especially for example to contribute to the structural integrity and structural resistance of a building. In contrast, slabs laid on the ground do for example not act as structural slabs. Slabs according to the present invention can thereby preferably be for example elevated slabs that are structural slabs.

In an embodiment of the invention, the supports may comprise columns, walls, piles or beams or any combination thereof or any other elements acting as vertical support, whereby further such supports can especially be point supports, linear supports or area supports.

In the present invention, the post-tension steel strands may be draped i.e. they are positioned for example to take away as much as possible the tensile stresses in the concrete, so that above the supports they are positioned in the upper half of the concrete slab and in-between the supports they are positioned in the lower half of the concrete slab.

In an embodiment of the invention, the post-tension steel strands may be in a banded-banded steel strands configuration or in a banded-distributed steel strands configuration or in a configuration resulting from any combination thereof, and/or the post tension steel strands can be arranged in any configuration, preferably without any maximum and/or minimum spacing requirements and/or the post-tension steel strand may be used for bonded or unbonded post-tensioning and/or the anchors for the post-tension steel strands may be designed as described for example in patent application US 63/052,283 so as to reduce bursting behind the post-tensioning anchors during or after post-tensioning and/or wherein the fibers are substantially homogenously or homogeneously distributed in the slab. A banded or banded-banded configuration of steel strands may thereby allow to keep the slab freer from steel strands, so as to allow.for example for more design freedom or safe drilling through the slabs. Bonded post-tensioning may thereby use bonded strands that may be bonded to the concrete of the slabs for example using grout, so that even in case of a problem an anchor structural integrity is preserved through the bonding.. On the other hand, unbonded post-tensioning strand may be provided with a plastic sheeting and may not be connected to the concrete of the slabs.

The supports may be arranged in a regular rectangular pattern or quadrilateral shape where a set of four supports or a set of four groups of supports forms a quadrilateral shape. The concrete slab comprises straight zones at the supports that connect the supports in the two directions, i.e. in length direction and in width direction, the shortest distance between those areas of the concrete slab above the supports. The straight zones have a width that may vary between 0 % and 80 %, e.g. between 5 % and 50 % of the greatest cross-sectional dimension of the slab width direction between two supports. Post-tension steel strands are present in bundles in those straight zones. The presence of bundles of post-tension steel strands in the straight zones is often referred to as banded pattern. Post-tension steel strands may or may not be present outside the straight zones.

In an embodiment, the supports may be arranged to form a regular rectangular pattern or quadrilateral shape, the concrete slab comprising straight zones connecting the supports via the shortest distance in two directions, i.e. lengthwise and width-wise, post-tension steel strand bundles being present only in said straight zones in closely-spaced arrangement, where for example the maximum distance between bundles may not exceed 0.8m, in a so-called banded-banded configuration, and/or the supports may be arranged to form a regular rectangular pattern or quadrilateral shape, the concrete slab comprising straight zones connecting the supports via the shortest distance in two directions, i.e. lengthwise and width-wise, post-tension steel strand bundles in any or both directions being present inside and/or outside said straight zones in a largely-spaced arrangement, where for example the maximum distance between bundles may exceed 1.5m, in a so called distributed or banded-distributed configuration. A bundle may thereby be a closely spaced arrangement, where two or more individual strands that may be arranged in close proximity to each other to form a bundle, whereby preferably the maximum distance between individual strands of a bundle may be < 0.8 m, further preferred < 0.25 m. As individual strands may be rarely used, as such, but may be more frequently used as part of a bundle, strands and bundles can be used interchangeably (or as synonyms) herein. A banded-distributed configuration is thereby achieved by having steel strand bundles arranged in a closely spaced arrangement one way i.e. in one direction (for example widthwise) and arranged in a largely spaced arrangement the other way i.e. in the other direction (for example lengthwise). Strands or bundles of strands can thereby be arranged especially for example in an arrangement selected from the group of: a two way distributed arrangement, a one way banded and one way distributed arrangement, a one way banded and one way mixed arrangement, whereby a mixed arrangement comprises both strands or bundles both in banded and distributed arrangements, a two way banded arrangement, a one way banded and one way mixed arrangement, whereby a mixed arrangement comprises both strands or bundles both in banded and distributed arrangements, a two way mixed arrangement, whereby a mixed arrangement comprises both strands or bundles both in banded and distributed arrangements.

In an embodiment, the slab and the supports may be either permanently fully connected, so that the slab is not free to move from its supports, permanently fully disconnected, so that the slab is free to move, partially connected, so that the slab is partially free to move in certain directions or temporarily disconnected, so that the slab is free to move at least temporarily until a connection is put in place. A disconnection or partial connection may thereby allow for example to reduce shortening restraint forces that may appear upon shrinkage and may lead to large cracks. This may be particularly useful for example for very stiff or very long slabs that may be particularly susceptible to shortening restraint forces for example due to the shrinkage of concrete, due to elastic shortening related to post-tensioning, due to creep of concrete or due to temperature changes. On the other hand, a connection may help to support higher loads, especially for example seismic loads.

In an embodiment, the span of the slabs between two supports for a given thickness is increased by between 5 and 50 %, preferably between 10 or 40 % or between 15 and 35 %, further preferred at least 5 %, 15 %, 20 %, 25 % or 30 % over a slab with the same slab thickness but without fibers and post-tension steel strands and/or wherein the thickness of the slab for a given span between two supports is reduced by between 5 and 50 %, preferably between 10 or 40 % or between 15 and 35 %, further preferred at least 5 %, 15 %, 20 %, 25 % or 30 % over a slab with the same span but without fibers and post-tension steel strands.

In an embodiment, the amount concrete can be reduced for a given thickness or a given span over a slab but without fibers and post-tension steel strands by between 5 and 50 %, preferably between 10 or 40 % or between 15 and 35 %, further preferred at least 5 %, 15 %, 20 %, 25 % or 30 %.

In an embodiment, the combination of post-tensioned steel strands and fibers may contribute to increases in the structural capacity for flexure, deflection, shear, punching shear, temperature resistance and/or resistance to shrinkage over a slab without steel fibers and/or steel strands. The present invention can thereby especially contribute to increase punching shear by for example 10 % to 100 %, preferably 20 % to 60 % compared to embodiments not according to the invention. Said combination can replace partially or totally any other form of steel reinforcement, and/or replace partially or totally over-thickening measures at supports such as for example drop cap or drop panel.

### Mode(s) for Carrying Out the Invention

### Explanation of the Principle behind the Invention

Concrete is a very brittle material that is hardly resistant to tensile tensions, the purpose is to avoid or at least to reduce the presence of tensile stresses.

Fig. 1 shows a schematic representation of a slab (1) on supports (2) with a draped post-tensioning steel strand (3) creating uplift forces (4) in-span and downward forces (5) at the supports (2), and concentrated loads (6) at the anchors.

Fig. 2a shows a concrete slab reinforced by means of a post-tension steel strand (7) that is located in the upper part of the slab. No external loads are present here. The post-tension steel strand (7) creates compressive stresses in the upper part of slab and tensile stresses in the lower part of slab. The ⊕ symbol, a plus sign in a circle, points to compressive stresses, while the e symbol, a minus sign in a circle, points to tensile stresses in Fig. 2 and Fig. 3.

Fig. 2b shows a schematic representation of a concrete slab with a negative applied moment represented by an arrow, which may represent the situation occurring for example at the supports. Compressive and tensile stresses resulting from the applied moment are show too.

Fig. 2c shows a schematic representation corresponding to Fig. 2b but where tensile stresses have now been reduced by the addition of the post-tensioning strand (7). This may especially allow to contribute to reduce or prevent the formation of cracks.

Fig. 3a shows a concrete slab reinforced by means of a post-tension steel strand (7) that is located in the lower part of the slab. No external loads are present here. The post-tension steel strand (7) creates compressive stresses in the lower part of slab and tensile stresses in the upper part of slab.

Fig. 3b shows a schematic representation of a concrete slab with a positive applied moment represented by an arrow, which may represent the situation occurring for example at in-span.

Fig. 3c shows a schematic representation corresponding to Fig. 3b but where tensile stresses have now been reduced by the addition of the post-tensioning strand (7). This may especially allow to contribute to reduce or prevent the formation of cracks.

In some embodiments, a post-tension steel strand may also be arranged in the middle of the slab.

However, no position can guarantee the total absence of tensile stresses. Within the context of the present invention, post-tension steel strands may therefore be designed especially for example to take up and compensate the tensile stresses that may originate during hardening and shrinkage of a concrete in addition to applied loads. The post-tension steel strands are of a sufficiently high tensile strength, i.e. above 1700 MPa or even above 1800 MPa, so that conventional concrete can be used and ingredients to compensate shrinkage can be avoided.

The fibers are mixed in the concrete as homogeneously as possible so that may preferably be present over the whole volume of the slab and able to take tensile stresses caused by various loads.

In a second embodiment of the invention, a concrete slab is formed on supports. A slip-sheet may be or may not be present between the supports and the slab.

### Post-Tension Steel Strand

A typical post-tension steel strand may have for example a 1+6 construction with a core steel wire and six layer steel wires twisted around the core steel wire. In an embodiment, the post-tension steel strand may be in a non-compacted form.

In an alternative preferable embodiment, the post-tension steel strand may be in a compacted form. In this compacted form, the six layer steel wires no longer have a circular cross-section but a cross-section in the form of a trapezium with rounded edges. A compacted post-tension steel strand has less voids and more steel per cross-sectional area.

As mentioned, the post-tension steel strand may have a high yield point, i.e. the yield force at 0,1 % elongation is high. The ratio yield force F_{p0,1} to breaking force Fₘ is higher than 75%, preferably higher than 80%, e.g. higher than 85%.

A typical steel composition of a post-tension steel strand is a minimum carbon content of 0,65%, a manganese content ranging from 0,20% to 0,80%, a silicon content ranging from 0,10% to 0,40%, a maximum sulfur content of 0,03%, a maximum phosphorus content of 0,30%, the remainder being iron, all percentages being percentages by weight. Most preferably, the carbon content is higher than 0,75%, e.g. higher than 0,80%. Other elements as copper or chromium may be present in amounts not greater than 0,40%.

All steel wires may be provided with a metallic coating, such as zinc or a zinc aluminium alloy. A zinc aluminium coating has a better overall corrosion resistance than zinc. In contrast with zinc, the zinc aluminium coating is temperature resistant. Still in contrast with zinc, there is no flaking with the zinc aluminium alloy when exposed to high temperatures.

A zinc aluminium coating may have an aluminium content ranging from 2 per cent by weight to 12 per cent by weight, e.g. ranging from 3 % to 11%.

A preferable composition lies around the eutectoid position: Al about 5 per cent. The zinc alloy coating may further have a wetting agent such as lanthanum or cerium in an amount less than 0,1 per cent of the zinc alloy. The remainder of the coating is zinc and unavoidable impurities.

Another preferable composition contains about 10% aluminium. This increased amount of aluminium provides a better corrosion protection then the eutectoid composition with about 5% of aluminium.

Other elements such as silicon (Si) and magnesium (Mg) may be added to the zinc aluminium coating. With a view to optimizing the corrosion resistance, a particular good alloy comprises 2 % to 10 % aluminium and 0,2 % to 3,0 % magnesium, the remainder being zinc. An example is 5% Al, 0,5 % Mg and the rest being Zn.

An example of a post-tension steel strand is as follows:
- diameter 15,2 mm;
- steel section 166 mm²;
- E-modulus: 196000 MPa;
- breaking load Fm: 338000 N;
- yield force F_{p0.1}: 299021 N;
- tensile strength Rm 2033 MPa.

### Steel Fiber

Steel fibers adapted to be used in the present invention typically have a middle portion with a diameter D ranging from 0,30 mm to 1,30 mm, e.g. ranging from 0,50 mm to 1,1 mm. The steel fibers have a length ℓ so that the length-to-diameter ratio ℓ/D ranges from 40 to 100.

Preferably, the steel fibers have ends to improve the anchorage in concrete. These ends may be in the form of bent sections, flattenings, undulations or thickened parts. Most preferably, the ends are in the form of three or more bent sections. In one embodiment, steel fibers may be glued.

Figure 4 illustrates a preferable embodiment of a steel fiber (8). The steel fiber (8) has a straight middle portion (9). At one end of the middle portion (9), there are three bent sections (10), (11) and (12). At the other end of the middle portion (9) there are also three bent sections (10'), (11') and (12'). Bent sections (10), (10') make an angle (a) with respect to a line forming an extension to the middle portion (9). Bent sections (11), (11') make an angle (b) with respect to a line forming an extension to bent sections (10), (10'). Bent sections (12), (12') make an angle (c) with respect to bent sections (11), (11').

The length ℓ of the steel fiber (8) may range between 50 mm and 75 mm and is typically 60 mm.

The diameter of the steel fiber may range between 0,80 mm and 1,20 mm. Typical values are 0,90 mm or 1,05 mm.

The length of the bent sections (10), (10'), (11), (11'), (12) and (12') may range between 2,0 mm and 5,0 mm. Typical values are 3,2 mm, 3,4 mm or 3,7 mm.

The angles (a), (b) and (c) may range between 20° and 50°, e.g. between 24° and 47°.

The steel fibers may or may not be provided with a corrosion resistant coating such as zinc or a zinc aluminium alloy.

In a particular preferable embodiment of the steel fiber, there are four bent sections at each end of the middle portion.

In another particular preferable embodiment of the steel fiber, the middle portion has an elongation at maximum load higher than 4%, e.g. higher than 5%, e.g. higher than 5,5%. Steel fibers with such a high elongation at maximum load may be used in structural applications such as floors on piles, elevated systems and structural wall systems.

### Macro-synthetic fiber

Examples of macro-synthetic fibers may be selected from carbon fibers, glass fibers, basalt fibers or other non-steel based fibers, such as fibers based upon polyolefins like polypropylene or polyethylene or based upon other thermoplastics.

### Arrangements

Fig. 5a shows a schematic representation of top down view of a two way distributed, namely for example lengthwise and width wise distributed, arrangement of strands or strand bundles (represented by lines). Supports are schematically represented as squares.

Fig. 5b shows a schematic representation of top down view of a one way banded and one way distributed arrangement of strands or strand bundles (represented by lines). Supports are schematically represented as squares.

Fig. 5c shows a schematic representation of top down view of a one way banded and one way mixed arrangement of strands or strand bundles (represented by lines), whereby a mixed arrangement comprises both strands or bundles both in banded and distributed arrangements. Supports are schematically represented as squares.

Fig. 5d shows a schematic representation of top down view of a two way banded arrangement of strands or strand bundles (represented by lines). Supports are schematically represented as squares.

Fig. 5e shows a schematic representation of top down view of a one way distributed and one way mixed arrangement of strands or strand bundles (represented by lines), whereby a mixed arrangement comprises both strands or bundles both in banded and distributed arrangements. Supports are schematically represented as squares.

Fig. 5f shows a schematic representation of top down view of a two way mixed arrangement of strands or strand bundles (represented by lines), whereby a mixed arrangement comprises both strands or bundles both in banded and distributed arrangements. Supports are schematically represented as squares.

### Examples of a Slab on supports

### First Example

- thickness of concrete slab: 0.2 m
- applied load:5 kN/m²
- distance between neighbouring supports: 7 m x 8.5 m
- type of support: columns
- distance between post-tension steel strands within the straight zones: 0.15 m
- not necessary that there are post-tension steel strands outside the straight zones, but in case there are post-tension steel strands, the distance between post-tension steel strands outside the straight zones is greater than 2.5 m, preferably greater than 1.5 m

### Second Example

- thickness of concrete slab: 0.15 m
- applied load: 2 kN/m²
- distance between neighbouring supports: 5 m x 5 m
- type of support: piles
- distance between post-tension steel strands within the straight zones: 0.15 m
not necessary that there are post-tension steel strands outside the straight zones, but in case there are post-tension steel strands, the distance between post-tension steel strands outside the straight zones is greater than 2.0 m, preferably greater than 1.5 m.

## Claims

1. A concrete slab resting on at least two supports, the slab comprising conventional concrete and a combined reinforcement of both draped post-tension steel strands and fibers,
said post-tension steel strands
- having a diameter ranging from 5 mm to 20 mm,
- having a tensile strength higher than 1700 MPa,
said fibers being either steel fibers and being present in a dosage ranging from 10 kg/m3 to 75 kg/m³ or being macro-synthetic fibers and being present in a dosage ranging from 1,5 kg/m³ to 9,0 kg/m³,
whereby the slab and the supports are fully connected, partially connected or fully disconnected.

2. The concrete slab according to claim 1,
wherein said conventional concrete has a characteristic compressive cube strength of 25 N/mm² or higher, preferably 28 N/mm² or higher, further preferred 30 N/mm² or higher and/or wherein the slab does not contain any further reinforcement elements, such as rebars or steel nets beside steel fibers and post-tensioning steel strands and/or wherein the slab is cast in one or multiple steps.

3. The concrete slab according to claim 1 or claim 2,
wherein said fibers are steel fibers or wherein the fibers are glued or wherein macro-synthetic fibers may be selected from carbon fibers, glass fibers, basalt fibers or other non-steel based fibers, preferably polyolefin fibers, further preferred polypropylene fibers or polyethylene fibers..

4. The concrete slab according to any of the preceding claims,
wherein said steel fibers comprise a straight middle portion that have a tensile strength above 1400 MPa, preferably above 1500 MPa, preferably above 1700 MPa, further preferred above 1900 MPa, even further preferred above 2000 MPa.

5. The concrete slab according to any of the preceding claims ,
wherein said steel fibers comprise anchorage ends at both ends,
said anchorage ends each comprise three or four bent sections and/or wherein said steel fibers have an elongation capacity of between 2.5 and 12 %, preferably at least 2.5%, preferably at least 3.5%, further preferred at least 4.5%, even more preferred a least 5.5 % and/or
wherein the slab comprising steel fiber concrete is strain hardening in bending.

6. The concrete slab according to any of the preceding claims,
whereby steel fibers are present in the slab in a dosage ranging from ≥ 25 kg/m³ to 60 or 65 kg/m³, preferably 20 kg/m³ to 30 kg/m³ or alternatively > 40 kg/m³ to 60 or 65 kg/m³.

7. The concrete slab according to any of the preceding claims,
wherein said supports are concrete supports, masonry supports, steel supports or supports combining concrete, masonry and/or steel and/or
wherein the supports are part of a foundation or preferably the supports are not part of a foundation.

8. A concrete slab according to any of the preceding claims, whereby the supports may comprise columns, walls, piles or beams or any combination thereof or any other elements acting as vertical support, whereby further such supports can especially be point supports, linear supports or area supports

9. A concrete slab according to any of the preceding claims,
whereby it further comprises plastic slip-sheets between said concrete slab and the supports, especially at the points of contact between the slab and the supports or whereby plastic slip-sheets are not present between the slab and the supports.

10. A concrete slab according to any of the preceding claims,
- wherein the post-tension steel strands are in a banded-banded steel strands configuration or in a banded-distributed steel strands configuration or in a configuration resulting from any combination thereof, and/or
- wherein the post tension steel strands can be arranged in any configuration, preferably without any maximum and/or minimum spacing requirements
- wherein the post-tension steel strand are used for bonded or unbonded post-tensioning and/or
- wherein the anchors for the post-tension steel strands are designed so as to reduce bursting behind the post-tensioning anchors during or after post-tensioning and/or
- wherein the fibers are substantially homogenously or homogeneously distributed in the slab.

11. The concrete slab according to any of the preceding claims,
wherein the slab and the supports are either permanently fully connected, so that the slab is not free to move from its supports, permanently fully disconnected, so that the slab is free to move, partially connected, so that the slab is partially free to move in certain directions or temporarily disconnected, so that the slab is free to move at least temporarily

12. The concrete slab according to any of the preceding claims
- said supports being arranged to form a regular rectangular pattern or quadrilateral shape, said concrete slab comprising straight zones connecting the supports via the shortest distance in two directions, i.e. lengthwise and width-wise, post-tension steel strand bundles being present only in said straight zones in a closely-spaced arrangement, where the maximum distance between bundles does not exceed 1.5m and/ or
- said supports being arranged to form a regular rectangular pattern or quadrilateral shape, said concrete slab comprising straight zones connecting the supports via the shortest distance in two directions, i.e. lengthwise and width-wise, post-tension steel strand bundles in one direction being present outside said straight zones in a largely-spaced arrangement, where the maximum distance between bundles exceed 1.5m.

13. The concrete slab according to any of the preceding claims,
wherein the span of the slabs between two supports for a given thickness is increased by between 5 and 50 %, preferably between 10 or 40 % or between 15 and 35 %, further preferred at least 5 %, 15 %, 20 %, 25 % or 30 % over a slab with the same slab thickness but without fibers and post-tension steel strands and/or
wherein the thickness of the slab for a given span between two supports is reduced by between 5 and 50 %, preferably between 10 or 40 % or between 15 and 35 %, further preferred at least 5 %, 15 %, 20 %, 25 % or 30 %.
over a slab with the same span but without fibers and post-tension steel strands.

14. The concrete slab according to any of the preceding claims,
wherein the amount of concrete can be reduced for a given slab thickness or a given span over a slab but without fibers and post-tension steel strands by between 5 and 50 %, preferably between 10 or 40 % or between 15 and 35 %, further preferred at least 5 %, 15 %, 20 %, 25 % or 30 %.

15. The concrete slab according to any of the preceding claims, wherein the combination of post-tensioned steel strands and fibers increases the structural capacity for flexure, deflection, shear, punching shear, structural integrity, temperature resistance and/or shrinkage resistance over a slab without steel fibers and/or steel strands.
